

May 10, 1938.

E. GERMER

2,116,927

ELECTRICAL DISCHARGE DEVICE

Filed April 13, 1937

Fig. 1



Fig. 3.



Edmund Germer  
INVENTOR

By  
Fried & Scherer, Attorneys  
ATTORNEYS

## UNITED STATES PATENT OFFICE

2,116,927

## ELECTRICAL DISCHARGE DEVICE

Edmund Germer, Berlin-Wannsee, Germany

Application April 13, 1937, Serial No. 136,540  
In Germany April 20, 1935

2 Claims. (Cl. 176—126)

This invention relates to electrical discharge devices and to electrodes adapted for use in such devices and to the method of producing and treating such electrodes. More particularly the invention relates to activated solid metallic electrodes 5 and to electrical discharge devices using such electrodes.

In an application of Hans J. Spanner, Serial No. 387,986, filed August 23, 1929, there is disclosed an activated electrode suitable for electrical discharge devices in which the electrode is subjected to ionic bombardment and in which, therefore, the activation of the electrode presents an especially difficult problem. It was there disclosed that in order to meet the requirements of this problem it is advantageous to have the surface of the metallic carrier on which the activation material is deposited as rough as possible. It was suggested in that application to obtain a rough surface by winding fine wire onto a core of heavy wire. It has also been suggested (e. g., in my German application, Serial No. 90,346, filed April 30, 1935) to produce such a surface by mechanically roughening the surface of the metallic carrier, e. g., by grooving, milling, etc.

It is an object of the present invention to provide a metallic carrier in an electrode structure with a roughened surface especially adapted for carrying activation material. Another object of the invention is to provide electrodes which may be more easily activated, which will have longer life and which in use will have more constant low electrode potential drop.

I have found that these objects can be best attained by an electrical treatment prior to activation.

According to my invention the metallic carrier before the activation treatment may be immersed in an electrolytic bath and subjected to an electrolytic treatment by which it is provided with a spongy metallic surface deposit in a manner well known in the art of electro-metallurgy.

Although I do not claim that such a spongy metallic surface deposit is in itself, unknown to the prior art, it is, so far as I am aware, unknown to utilize such a deposit in electrodes for discharge devices and especially for holding the activation on the electrodes. Such deposits have been known in the art of electro-metallurgy as the result of defective conditions and to be avoided; but I have now discovered that the result thus produced is superior for the purposes of electrode activation to the surfaces which could be obtained in other ways.

In one example of my invention a suitable me-

tallic electrode structure (e. g., a cylinder for radio tubes, spiral wire or sheet metal, cups, cylinders or discs for gaseous discharge tubes, etc.) before the application of the activating material is treated in an electrolytic bath. Using, for example, as the base metallic structure nickel, tungsten or molybdenum, a nickel plating bath is preferably chosen. For best results the strength of the electrolytic current is chosen so that the electrode to be treated is greatly overloaded. Thus, a coating forms on the electrode surface which is not a smooth dense plating but which has a microporous surface (commonly known as nickel sponge, etc.).

After the treatment of the electrode by which this porous surface is produced, it is degassed by heating in vacuum or in an atmosphere of inert gas to drive off any objectionable occluded gases and to reduce any objectionably oxidized material; and the activating mass is coated onto the porous surface; and, finally, the electrode thus coated is again subjected to degassing and/or reduction in vacuo and/or to any other desired activation treatments such as are now well known in the art.

In some cases it may be preferable to apply the activation material before the electrode base is cleaned and directly after its electrolytic treatment. In general, however, this is not to be recommended, since the elimination of gas from the porous structure may tend to loosen the applied coating of activation material.

Instead of a single application of metal deposits, this may be changed with advantage in some cases so that it is treated in several baths, e. g., to produce successive coatings of different micro-structure and/or of different metals.

Thus, for example, the electrode referred to above after coating with the porous nickel can be subjected to a second chromium plating bath in which the electrode is similarly overloaded so as to produce a micro-porous deposit of chromium.

Also the intensity of the current during the treatment may be changed so that the character of the coating is changed throughout its thickness. Thus it is particularly advantageous to start with a normal plating current and gradually to increase the current, thereby increasing gradually the porosity of the applied coating

A similar favorable effect may be attained also if the metal structure to be treated is connected in the electrolytic bath, not as a cathode, but as an anode. In this case with a heavy overloading of the electrolytic current the surface of the

dense metal is loosened up so that after the treatment similar favorable effects are found. In this way it is possible to treat electrodes in the same bath both at the anode and at the cathode.

5 As examples of my invention I may take a spiral tungsten wire about approximately 3 mills diameter, e. g., of the form shown in Fig. 1, and connect this as the cathode in a plating circuit and immerse it in a plating bath containing 227 10 grams nickel ammonium sulfate, 57 grams ammonium sulfocyanate, 28 grams zinc sulfate, 4.5 liters water and having a strength of about 6° Baumé and a temperature of about 27° to 30° C.

This bath may, of course, also contain other ingredients, as is well known in the art of electro-plating. As anode a nickel bar is immersed in the bath and connected into the plating circuit. Through this circuit is passed a current of about 0.02 amp. with a voltage of about 1 volt. This 15 current is continued for about 1 hour after which the electrode is removed from the bath, dried, placed in the vacuum chamber and heated to a glowing temperature, meanwhile exhausting the vacuum chamber to remove the gases released 20 from the metal. The electrode after cooling, and preferably with little or no exposure to the air, is immersed in a suspension or paste of 50 parts of barium oxide, 30 parts of strontium oxide and 20 parts of calcium oxide, all in finely divided state 25 and suspended in a thin solution of collodion. After this dipping, the electrode is dried and may be dipped again or several times with drying after each. It is then sealed into the tube in which it is to be used and is again subjected to 30 vacuum and heating treatments, e. g., by high frequency bombardment, to decompose the collodion and drive off any occluded gases, and if desired to reduce partially or to any desired extent the activating oxides; and finally, is subjected to a discharge in the tube, preferably before the final pumping and sealing off of the tube. 35

As a second example, an electrode structure, e. g., as shown in any of the figures of the drawing, may be connected into a plating circuit and immersed in an ordinary plating bath, e. g., the nickel plating bath as described in the first example (in which case the electrode structure is itself preferably of nickel), and the plating circuit connected so that the electrode is the anode in the bath. It is then subjected to a current of 40 approximately 0.05 amp. at 2 volts for a period 45

of 1 hour. When removed it will have a desired porous structure and may then be subjected to further treatment substantially as described in connection with the first example.

As another example, the electrode may be 5 treated as in the first example, except that instead of subjecting it to a uniform current throughout its treatment the treatment may be started with a current of 0.015 amp. and increase 10 gradually over a period of ½ hour until it reaches a current of 0.25 amp. The treatment may then be continued for ¼ hour with said current, after 15 which the electrode is removed and may be subjected to the same cleaning and activation treatment as before described. 15

In the drawing, I have shown in Fig. 1 a longitudinal section through a discharge lamp embodying my invention.

In Fig. 2, I have shown in elevation another type of electrode adapted to be directly heated 20 to thermionic temperature by a resistive current; and

In Fig. 3, I have shown a third type of electrode, namely an indirectly heated uni-potential cathode partly in section and partly in elevation. 25

In all of these figures, I have indicated the electrode structure proper or carrier metal by the reference character 10, 10a, 10b, the lead-in wires by the reference characters 11, 11a and 11b; and the porous metal coating with its adhering activation layer, by the reference character 12. 30

What I claim is:

1. An electrode for an electric discharge tube which comprises a dense metal carrier base, an integral metallic surface layer thereon, more porous than the base, and a coating of activation material adhering to said porous layer, the outer layer of metal on said electrode being of gradually increasing porosity as the activated surface of the electrode is approached. 40

2. The method of treating a metallic electrode by connecting it as an electrode in an electrolytic bath and subjecting it to a substantial overload current, whereby the metal at its surface is given a porous structure, and thereafter cleaning it to remove impurities and occluded gases in which the electrolytic treatment is started with the current adapted to leave a dense metal surface and is gradually increased to an overload current adapted to produce a spongy surface. 45

EDMUND GERMER. 50